

Aug. 2, 1932.

O. W. ELLIS

1,869,554

ALLOY

Filed Dec. 14, 1928

Fig. 1.



Fig. 2.



INVENTOR

Owen W. Ellis.

BY  
Chester G. Barr  
ATTORNEY

## UNITED STATES PATENT OFFICE

OWEN W. ELLIS, OF PITTSBURGH, PENNSYLVANIA, ASSIGNOR TO WESTINGHOUSE ELECTRIC & MANUFACTURING COMPANY, A CORPORATION OF PENNSYLVANIA

## ALLOY

Application filed December 14, 1928. Serial No. 326,029.

My invention relates to alloys and more particularly to an aluminum brass in which iron and manganese have been substituted for part of the zinc.

5 An object of my invention is to provide an improved aluminum brass having an alpha beta or a beta structure that has greater ductility and strength than previous alloys of this type.

10 Another object of my invention is to provide an improved aluminum brass having an alpha beta or a beta structure in which iron, or a mixture of manganese and iron, has been substituted for part of the zinc in the 15 brass in such proportions that the ductility of the alloy is increased without causing a decrease in its strength.

15 A further object of my invention is to provide an improved aluminum brass having an alpha beta or a beta structure in which manganese, or a mixture of manganese and iron, has been substituted for the zinc in such proportions that the strength of the alloy is increased without causing a decrease 20 in its ductility.

Brass composed of 64 to 54% copper and from 46 to 36% zinc, crystallizes upon cooling in the alpha beta structure, while brass containing between 46 and 50% zinc and from 25 54 to 50% copper crystallizes upon cooling in the beta structure. It is a well known fact that the substitution of aluminum for part of the zinc in a brass having an alpha beta or a beta structure causes an increase 30 in strength and a decrease in ductility. Such a substitution also reduces the amount of the alpha constituent in a brass having an alpha beta structure and if sufficient quantities are added, the alpha constituent can be entirely eliminated. This also has the tendency to reduce the ductility of the alloy because brass having an alpha beta structure is usually 35 more ductile than brass having a beta structure. It will, therefore, be understood that the increase in strength that can be produced by the substitution of aluminum for part 40 of the zinc in a brass is largely, if not completely, determined by the ductility required. As a general rule, the aluminum content of the brass should not exceed 5%.

In order to further increase the strength of an aluminum brass, it has heretofore been proposed to substitute manganese and iron for part of the zinc, and alloys comprising copper, zinc, aluminum, iron and manganese 55 are well known. In making a thorough investigation of the alloys of this type, however, I have found that the substitution of iron and manganese for part of the zinc in an aluminum brass having an alpha beta or 60 a beta structure is not always beneficial because the addition of these ingredients in different proportions causes widely divergent results. For example, when they are added in certain proportions they cause a decrease in both the strength and ductility of the 65 alloy. Other proportions increase the strength of the alloy but reduce the ductility, or, conversely, increase the ductility but reduce the strength.

I have made the discovery that when certain well defined proportions of iron and manganese are substituted for a part of the zinc in an aluminum brass substantially free from all but accidental traces of tin and having an alpha beta or a beta structure, an alloy 70 will be produced that is improved both in ductility and strength. The proportions of iron and manganese may also be varied so that an increase in strength may be produced without affecting the ductility of the alloy, or an increase in ductility may be produced without affecting the strength.

75 My invention will be better understood by reference to the accompanying drawing in which:

Figure 1 is a graph showing the proportions of iron and manganese which, when substituted for part of the zinc in an aluminum brass, increase the ductility without 80 decreasing the strength, and

Fig. 2 is a graph showing the proportions of the same ingredients which, when substituted for a portion of the zinc in a similar brass, increase the strength without reducing 85 the ductility.

90 Referring to Fig. 1 of the drawing, the ordinates indicate the percentage of iron and the abscissæ the percentage of manganese to be substituted in the alloy. The dotted line 1 95

designates the increase in percentage elongation in two inches obtained in an aluminum brass having an alpha beta or a beta structure when iron and manganese have been 5 substituted for a part of the zinc in the brass in the proportions designated by the heavy line 2. While the substitution of iron and manganese for part of the zinc in the alloy in the proportions indicated by the line 2 10 produces an alloy having increased ductility, the tensile strength of the alloy is not decreased.

The graph shows that an increase in ductility, as measured by percentage elongation 15 in two inches, may be obtained without loss of strength, when the proportion of iron in the alloy is varied between about 1.25% and 4.8% and the proportion of manganese between 0 and 5%. 20 It will be noted that when about 1.6% iron and about .7% of manganese are substituted for 2.3% of zinc in an aluminum brass, the ductility of the alloy as measured by percentage elongation in two inches will be 25 approximately 11% greater than that of ordinary aluminum brass. For example, an aluminum brass composed of 58% copper, 2% aluminum and the balance zinc, was tested. The tensile strength of the alloy was 30 87,000# per square inch and the percentage elongation was 21% in two inches. Iron in the proportion of 1.6% and manganese in the proportion of 0.7% were then substituted for 2.3% of the zinc and the resulting alloy, 35 consisting of: 58% copper, 2% aluminum, 1.6% iron, 0.7% manganese, balance zinc, had a tensile strength of 87000# per square inch and a percentage elongation of 32% in two inches.

40 Referring to Fig. 2 of the drawing, the ordinates and abscissæ indicate the percentages of iron and manganese, respectively, the heavy line 3 the percentages of manganese and iron that may be substituted in an aluminum brass for a part of the zinc without 45 causing a decrease in ductility, and the dotted line 4 the increase in tensile strength that is effected by this substitution. It will be noted from this graph that when iron and manganese are substituted for zinc in an aluminum brass having an alpha beta or a beta structure in a range of proportions between 50 0 and 2% iron, and between 2 and 7% manganese, an improved alloy will be produced 55 that has a greater tensile strength than an ordinary aluminum brass, and is equally as ductile.

While the proportions of iron and manganese represented by any point on the heavy 60 line 3 in Fig. 2 of the drawing may be utilized, it is apparent that good results may be produced by substituting about 1% iron and about 3.65% of manganese for 4.65% of zinc in an aluminum brass having an alpha beta or a beta structure, and that the increase in

tensile strength which is obtained by making a greater substitution is very limited. When iron and manganese in the proportions just specified were substituted for 4.65% zinc in an aluminum brass containing 58% copper, 2% aluminum and the balance zinc, an alloy was produced having the following composition: 58% copper, 2% aluminum, 1% iron, 3.65% manganese, balance zinc. This alloy had a tensile strength of 93,700# per square 70 inch while the tensile strength of the original alloy was only 87,000#. The ductility of the two alloys, as determined by the percentage of elongation, was practically the same.

Since the proportions of iron and manganese that are effective in causing an increase in ductility without causing a decrease in strength range from 1½ to 5% iron and from 0 to 5% manganese and the proportions of the same ingredients that cause an increase in 80 strength without causing a loss in ductility range from 0 to 2% iron and 2 to 7% manganese, it will be obvious that when the proportions of iron and manganese are maintained within the limits of 1½ to 2% iron and 90 2 to 5% manganese, alloys having both an increased strength and ductility will be produced.

It will be recognized that in practice, it is difficult to produce an alloy having the exact 95 percentages represented by the heavy lines 2 and 3 in Figs. 1 and 2 and where specific proportions of the ingredients are mentioned in the claims, it is contemplated that there may be some variations in manufacture, such as an 100 increase or decrease of about .25% of either or both the manganese and iron.

While I have described a preferred embodiment of my invention and have illustrated by examples and graphs the proportions of iron and manganese, which when substituted for zinc in an aluminum brass having an alpha beta or a beta structure, produce an alloy having the desired characteristics, it will be understood that various modifications may be made therein without departing from the spirit of my invention.

For example, the aluminum content may be varied from 0 to 5% and the iron and manganese may be varied within those ranges that will produce an alloy having increased strength and ductility, an increased ductility without a decrease in strength, or an increase in strength without loss in ductility. It will also be understood that varying amounts of impurities may be present in the alloys. It is essential however that the proportion of tin should be kept below a range of .5 to .75% because of its deleterious properties.

Other modifications of my invention will be apparent to those skilled in the art. I, therefore, desire that only such limitations shall be imposed thereon as are required by the prior art and the appended claims.

I claim as my invention:

1. An alloy comprising zinc, copper, aluminum, iron and manganese that is substantially free from tin, the zinc, copper and aluminum being present in such proportions that the alloy will crystallize in the alpha beta or beta structure, the proportion of iron being less than 2% and the proportion of manganese being less than 2.5%.
- 10 2. An alloy comprising zinc, copper, aluminum, iron and manganese that is substantially free from tin, the zinc, copper and aluminum being present in such proportions that the alloy will crystallize in the alpha beta or beta structure, the proportion of iron being greater than .75% but less than 2% and the proportion of manganese being less than 2.5%.
- 15 3. An alloy comprising zinc, copper, aluminum, iron and manganese that is substantially free from tin, the zinc, copper and aluminum being present in such proportions that the alloy will crystallize in the alpha beta or beta structure, the proportion of iron being at least 1% but less than 2%, and the proportion of manganese being less than 2.5%.
- 20 4. An alloy comprising zinc, copper, aluminum, iron and manganese, the zinc, copper and aluminum being present in such proportions that the alloy will crystallize in the alpha beta or beta structure, the amount of iron being greater than .75% but less than 2%, the amount of aluminum being less than 5% and the amount of manganese ranging from .25% to 2%.

In testimony whereof, I have hereunto subscribed my name this 12th day of December, 1928.

OWEN W. ELLIS.

40

45

50

55

60

65